# EUROPEAN PATENT SPECIFICATION

(11) **EP 0 839 891 B1**
(45) Date of publication and mention of the grant of the patent: **16.06.2004**
(21) Application number: 97500182.7
(22) Date of filing: 30.10.1997
(51) Int. Cl.: C10G 21/28, C09D 11/02, C08K 5/01, C08L 21/00

(54) **Process for obtaining aromatic oils having a polycyclic aromatics content of less than 3% which are useful as process oils**
Verfahren zur Herstellung von Ölen mit einem Gehalt an polycyclischen Aromaten von weniger als 3%, verwendbar als Prozessöle
Procédé pour l'obtention d'huiles à teneur en aromatiques polycycliques de moins que 3% utilisables comme huiles de procédé

(30) Priority: 31.10.1996 ES 9602311; 28.10.1997 ES 9702226
(43) Date of publication of application: 06.05.1998
(73) Proprietor: REPSOL PETROLEO S.A., E-28046 Madrid (ES)
(72) Inventor: Moreno, Rodriguez, Juan Miguel, 28047 Madrid (ES); Monjas, Serrano, Carlos, 28035 Madrid (ES)
(74) Representative: Davila Baz, Angel

(56) References cited:
- EP-A- 0 043 267
- EP-A- 0 362 446
- EP-A- 0 417 980
- FR-A- 2 685 705

## Description

### Scope of the invention

This invention relates to a new process for obtaining aromatic oils having a polycyclic aromatic (PCA) compounds content of less than 3% (IP-346), the aromatic oils so obtained and their application as process oils, such as rubber extenders and oils for printing inks.

### Background to the invention

The components used in the manufacture of rubber, especially in the application for pneumatic tyres, include aromatic oils.

At the present time these aromatic oils are obtained as a by-product of the process of solvent extraction (basically using phenol, furfural, and N-methyl pyrrolidone) of vacuum distillates used as a raw material for the manufacture of lubricant base oils. These aromatic oils, also known as DAE (distillate aromatic extracts) have as a main disadvantage their carcinogenicity due to the polyaromatic hydrocarbons (PAH) and polyaromatic compounds (PAC) which they contain. The latter are found in concentrations very much in excess of 3% (IP-346), the value above which these compounds are regarded as being potentially carcinogenic.

In order that a process oil should behave efficiently it is essential that it should have suitable miscibility and solvent properties. In the case of rubbers having a significant percentage of aromatic groups, such as styrene-butadiene (SBR), aromatic oils (DAE) having an aromatic hydrocarbons content in excess of 70% (generally in the range 70-85%) are used, but with a PAC content of around 15% by weight (IP-346).

Another important aspect of the aromatic oils used in the manufacture of rubber is their volatility, which if high leads to the emission of smoke during the manufacturing process.

On the other hand, the use of aromatic oils in the formulations of printing inks is limited to products that can not be labeled as potentially carcinogenic.

There is therefore a need to develop low volatility aromatic oils having a lower PAH content and a PAC content (IP-346) below 3% which can replace present oils, eliminating the problem of their potential carcinogenicity.

### State of the art

As already mentioned, the aromatic oils currently in use are obtained as a by-product in the manufacture of lubricant base oils during solvent extraction of the various vacuum distillates and the deasphalted vacuum bottoms obtained from reduced crude.

The following are obtained as a result of the extraction process: a flow rich in saturated hydrocarbons having a small solvent content known as mixed raffinate, which is the raw material for the manufacture of lubricant base oils, and a flow known as the mixed extract which mainly consists of solvent and oil rich in aromatic hydrocarbons.

The mixed extract flow is passed to a system for the recovery of solvent which is recycled to the extraction column, and an aromatic oil is obtained having a composition which depends on the nature of the vacuum distillate, the conditions under which extraction took place and the efficiency of the extraction column.

In general, for these extracts to be used as a process oil a high content of aromatic hydrocarbons is required, and this is generally above 75% by weight (ASTM D-2007). These aromatic extracts (DAE) obtained from vacuum distillates have a polyaromatic compounds (PAC) content in excess of 3%, with the result that they are regarded as being potentially carcinogenic. The aromatic extracts obtained from deasphalted vacuum bottoms have a PAC content which may be in excess of 3%, but despite this they cannot be regarded as potentially carcinogenic.

In European patent EP-A-417 980 a process for obtaining oils with a PAC content of less than 3% is described. The process consists of countercurrent reextraction of the primary extract obtained in the manufacture of lubricant base oils. The extract used as a feed to the reextraction column preferably contains not more than 20% by volume of solvent. This process therefore assumes that most of the solvent will be removed, so that it is then added at the reextraction stage. The quantity of additional solvent required varies between 1 and 1.8 times the quantity of extract being treated. On the other hand, in this application there is no reference to other characteristics such as PAH content, mutagenicity index or volatility of the new process oils.

### Summary of the invention

A process has now been found which can be used to obtain aromatic oils having a PAC content of less than 3% starting from the mixed extract flow obtained in the process for the manufacture of lubricant base oils described above.

The process according to this invention can bring about a considerable reduction in polyaromatic hydrocarbons (PAH) content in accordance with US standard EPA-8270 in comparison with the extracts in the state of the art.

The products obtained according to the invention are of a predominantly aromatic nature, with an aromatic hydrocarbons + polar compounds content of more than 45% according to ASTM D-2007, and preferably within the range 60 - 90%.

As a result of the process according to the invention the aromatic oils obtained cease to be regarded as potentially carcinogenic and can be used among other applications as extender oils for rubber or in formulations for printing inks.

### Basis of the invention

This invention is based on the following grounds:
1. The solvents used in the manufacture of lubricant base oils which constitute the majority component of the flow known as the mixed extract are solvents having great selectivity for polyaromatic compounds.
2. The selectivity and capacity of a solvent vary with:
   a) The solvent/solute ratio
   b) Temperature: in general, as the temperature decreases selectivity increases and dissolving power decreases.
   c) The addition of anti-solvents which regulate dissolving power and can increase selectivity. A typically used anti-solvent is water.
   d) Use of counter-solvents: these are compounds which act together with the solvent modifying the phase equilibrium. Typical counter-solvents used are e.g. light paraffins.

### Advantages of the invention with respect to the state of the art

The advantages of the new process according to this invention in comparison with the said European patent EP-A-417 980 are as follows:
1. Direct use of the mixed extract flow with a consequent reduction in the quantity of additional solvent:
   a) In the case of extract from deasphalted vacuum bottoms no additional solvent is required,
   b) In the case of SN-500 or heavier extracts, the quantity of additional solvent will always be less than 1:1 (with reference to the aromatic oil contained in the mixed extract),
   c) If the extracts are originated from bases of lower viscosity, the quantity of additional solvent will always be less than 1.5:1 (with reference to the aromatic oil contained in the mixed extract) and generally less than 1:1.
2. Use of anti-solvents and counter-solvents to improve selectivity for polyaromatic components. In this case the quantity of additional solvent will be greater than when no anti-solvents or modifiers are used.
3. Possibility of adding a hydrocarbonated stream with an initial boiling point at atmospheric pressure, greater than 200°C, preferably greater than 300°C, which allows increasing the production capacity of aromatic oils low in PCA content.
4. Reextraction of the extracts to obtain process oils should be performed with the purpose of removing polyaromatic compounds while maintaining the maximum concentration of mono and diaromatic compounds. Very low temperature conditions and solvent/extract ratios may be required in order to achieve this selectivity, and this might give rise to hydrodynamic problems in a countercurrent operation with very aromatic high viscosity extracts. The various modes of operation described in this invention overcome this problem:
   a) Non-use of countercurrent extraction for heavier extracts, or
   b) Use of counter-solvents which reduce viscosity and ensure that the countercurrent operation is performed correctly.
5. Another advantage of the process according to this invention is excellent characteristics as regards PAH content, mutagenicity index and volatility no reference to which is made in the above mentioned European patent application.

### Objects of the invention

Firstly the invention provides a process for obtaining aromatic oils from the mixed extract flow obtained in the manufacture of lubricant base oils, a flow which contains a polar solvent, preferably of the group comprising phenol, furfural and N-methyl-2-pyrrolidone, preferably furfural, characterized in that it comprises the stages of:
a) cooling the flow of mixed extract to render non-polyaromatic components insoluble,
b) settling to bring about separation of the phases,
c) conducting the heavy phase obtained from the settling in step b) to a solvent recovery system,
d) total or partial redissolution in solvent of the light phase obtained from the settling in stage b),
e) cooling to effect separation of the non-polyaromatic components,
f) settling to bring about separation of the phases,
g) conducting the heavy phase obtained from the settling in step f) to the solvent recovery system of step c)
h) recovering the light phase having a low polyaromatic compounds content obtained from the settling in step f),
i) passing said light phase to a system for the recovery of the solvent, and
j) recycling the solvent recovered in steps c), g) and i) to the process.

Secondly , the invention provides a process for obtaining aromatic oils with a polycyclic aromatic compounds content of less than 3% (IP-346) from the mixed extract flow, originating from the solvent extraction of a deasphalted vacuum bottom, obtained in the manufacture of lubricant base oils, a flow which contains a polar solvent in a rate between 70 and 95 %, preferably of the group comprising phenol, furfural and N-methyl-2-pyrrolidone, preferably furfural, characterized in that it comprises the stages of:
a) cooling the flow of mixed extract to render non-polyaromatic components insoluble,
b) settling to bring about separation of the phases,
c) conducting the heavy phase obtained from the settling in step b) to a solvent recovery system,
d) passing directly the light phase obtained in step b) to a system for the recovery of the solvent, and
e) recycling the solvent recovered in steps c) and d) to the process.
f) Lower viscosity than, but volatility similar to the aromatic oils in the state of the art,
g) Aromatic hydrocarbons + polar compounds content more than 45% (ASTM D-2007) and preferably in the range 60 - 90%.

Aromatic oils which can be regarded as being without carcinogenic potential, obtained in accordance with the process of the first or second feature of the invention from aromatic extracts obtained from vacuum distillates or deasphalted bottoms, have the following characteristics:
a) Viscosity at 100°C within the range 2 - 70 cSt,
b) Viscosity indexes generally below 75 in oils having a viscosity of more than 12 cSt (100°C),
c) PAC content less than 3% by weight (IP-346),
d) Lower polyaromatic hydrocarbons (PAH) content (US EPA-8270) than the aromatic extracts in the state of the art,
e) Mutagenicity index according to the modified Ames test (ASTM E-1687-95) very much less than 1,

Said low PAC content aromatic oils which can be regarded as being without carcinogenic potential, obtained according to the invention, can be used as process oils such as extenders for rubber, and oils for printing inks.

Rubbers having a high percentage of aromatic groups, such as styrene-butadiene rubbers, can be extended with the aromatic oils obtained according to the invention.

### Embodiments of the process according to the invention

In the process according to the invention an anti-solvent, for example water, can optionally be added to the flow of starting mixed extract in order to increase selectivity for PCAs, in quantities between 0.5 and 10%, preferably between 0.5 and 5% and in particular between 1 and 2.5%.

An important aspect of the process according to the invention is that the quantity of additional solvent in relation to the flow of the hydrocarbon phase in the mixed extract flow is always less than 1.5:1 and preferably less than 1:1.

In addition to this, and optionally, part of the solvent contained in the flow of starting mixed extract can be removed before the cooling stage in order to achieve an approximately 50% distribution of solvent in the stages prior to settling, or add a hydrocarbonated phase with an initial boiling point (IBP) greater than 200°C, preferably greater than 300°C, to regulate the solvent/solute rate and increase the production capacity of aromatic oils with a PCA content below 3%.

Likewise, and optionally, a counter-solvent can be added before the first cooling stage in order to increase the selectivity of the solvent contained in the mixed extract flow. Preferably the said counter-solvent may be a hydrocarbon flow with a maximum boiling point of less than 160°C, preferably less than 140°C.

The cooling temperature prior to the settling stages lies within the range 10 - 90°C, preferably within the range 10 - 60°C and in particular within the range 20 - 50°C.

In the case of aromatic extracts originating from deasphalted vacuum bottoms it may not be necessary to add additional solvent.

### Brief description of the appended drawings

The process according to the invention can be better understood with reference to the following detailed description thereof in combination with the appended drawings, in which:

Figure 1 is a flow diagram of the process according to the state of the art for obtaining aromatic oils as by-products in the production of lubricant base oils during the solvent extraction of various vacuum distillates and the deasphalted vacuum bottom obtained from reduced crude.

Figure 2 is a flow diagram of the process according to this invention for obtaining aromatic oils with a PAC content of less than 3% from the flow of mixed extract according to the state of the art, in which the process is based on the alternatives of reducing the temperature of the mixed extract flow and the optional addition of an anti-solvent, or of a hydrocar-bonated stream with IBP greater than 200°C.

Figure 3 is a flow diagram of the process according to the invention for obtaining the said aromatic oils, in which the process is based on the alternatives of reducing the temperature of the mixed extract flow and adding a counter-solvent.

### Detailed description the invention

For comparative purposes Figure 1 shows a flow diagram of the process according to the state of the art used for the production of aromatic extracts.

With reference to the said Figure 1, vacuum distillate (2) and extraction solvent (1) are placed in countercurrent contact in column C-1. The most frequently used solvents are: phenol, furfural and N-methyl-2-pyrrolidone. Solvent (1), which is of greater density, is added to the column at a point close to the top, and distillate (2), of lower density, is introduced at a point close to the bottom. The extraction column may be of various types although one of the most widely used is a mechanically stirred column. In the zone between the two inlet points, countercurrent contact takes place between the solvent and the vacuum distillate. As the solvent flows down the column it will become richer in the aromatic components for which it is most selective. At the same time the rising hydrocarbon flow becomes enriched in saturated hydrocarbons. In general the column operates with a certain temperature gradient which makes it possible to achieve a greater efficiency in the flow which is rich in saturated hydrocarbons. For this purpose part of the descending flow (4) is removed from the column, generally at a point below that at which vacuum distillate enters, and is cooled in an external exchanger (E-1) returning to the column (C-1) via (5).

The extraction process yields a flow rich in saturated = hydrocarbons with a small solvent content (3), known as mixed raffinate, which passes to the recovery system (SR-O) and constitutes the starting material for the manufacture of lubricant base oils, and a flow known as the mixed extract (6), which is predominantly made up of solvent and oil rich in aromatic hydrocarbons.

The flow of mixed extract (6) is passed to a solvent recovery system (SR-3) which recycles to the extraction column (C-1) and an aromatic oil (28) is obtained whose composition depends on the nature of the vacuum distillate, the conditions under which extraction took place and the efficiency of the extraction column.

The aromatic extracts obtained in accordance with this process according to the state of the art have a polyaromatic compounds (PAC) content of more than 3%, as a result of which they are regarded as being potentially carcinogenic.

With reference now to Figure 2, this shows the flow diagram of the process according to the invention based on cooling of the starting mixed extract flow and the optional addition of an anti-solvent, or of a hydrocarbonated stream with IBP greater than 200°C.

Specifically, Figure 2 shows a flow diagram of the process according to the invention for obtaining aromatic oils having a PAC content of less than 3% from the mixed extract flow according to the state of the art (6) by cooling in E-2 (and optionally by the addition of water, or of a hydrocarbonated stream with IBP greater than 200°C (7)), and settling in D-1. The light phase (12) obtained in D-1 is mixed with additional solvent at a higher temperature (14) to achieve satisfactory contact between the phases in mixer M-2 and partial or total redissolution. The new flow, 16, is again cooled in exchanger E-4 and is fed to settler D-2 where a new light phase (18) separates out and is sent to a solvent recovery system (SR-2). Flow (22), which is solvent-free, has a PAC content of less than 3% by weight.

If the flow of mixed extract is originated from the solvent extraction of a deasphalted vacuum bottom, then the light phase obtained in settler D-1 can be passed directly to solvent recovery (SR-2), as this flow has a PAC content of less than 3%.

Optionally the flow of mixed extract (6) can be passed to a solvent recovery system (SR-1) to remove some of the solvent before the stage of cooling and settling in D-1. The solvent removed in SR-1 is passed together with the additional solvent required for mixing with the light flow from D-1 for further reextraction and settling in D-2.

### Operating conditions of the process according to the flow diagram in Figure 2

Flow (6) leaves column C-1 at a temperature which generally varies within the range 50 - 115°C. This flow has a solvent content which likewise varies within the range 70 - 95%, most frequently being 80-85%. The oil contained in this flow has a polyaromatic hydrocarbons content which varies within the range 4 - 30%. This flow is cooled to a temperature within the range 10 - 90°C, preferably 20 - 50°C, in exchanger E-2. The cold flow from E2 is passed to settler D-1, where a light phase (12) having a low solvent content and a PAC content in the range 0.5 - 10%, fundamentally depending on the type of vacuum distillate (2), separates out. The light flow leaving D-1 is mixed (M-2) with solvent at a higher temperature within the range 30 - 160°C to dissolve most of the hydrocarbon components and is again cooled to the desired settling temperature, generally within the range 10 - 90°C and preferably within the range 20 - 50°C, in exchanger E-4. The cold flow (17) is passed to settler D-2 where a light phase (18) having a low solvent and polyaromatic compounds content again separates out. Flow (18) is passed to system SR-2 for the removal of the solvent. Optionally, an anti-solvent (7) or a hydrocarbonated fraction with IBP greater than 200°C (7), may be added to the mixed extract flow, which, in order to simplify, have both been considered as the same stream in fig. 2.

With reference now to Figure 3, this illustrates the process according to the invention based on cooling of the starting mixed extract flow and the addition of a counter-solvent.

Specifically, Figure 3 shows the flow diagram for the process based on temperature reduction, the addition of a counter-solvent and reextraction.

A counter-solvent (7) is added to the flow of mixed extract (6), and the resulting flow is cooled in exchanger E-2. The resulting flow (9) is passed to a mixer M-1 in order to achieve a satisfactory level of contact between the phases and then to a settler, D-1, where the phases separate out. The light phase (12) is mixed with additional solvent (14) in a mixer M-2, and is again cooled in exchanger E-4, from which it passes to settler D-2. The light phase (18) leaving D-2 is passed to a system SR-2 for the recovery of solvent and counter-solvent which are recycled to the process and a flow (22) having a PAC content of less than 3% is obtained.

If the flow of mixed extract originates from the solvent extraction of a deasphalted vacuum bottoms then the light phase obtained in settler D-1 can be passed directly to solvent recovery SR-2 if its PAC content is less than 3%.

Optionally the flow of mixed extract (6) can be passed to a solvent recovery system (SR-1) to remove part of the solvent before the stage of cooling and settling in D-1. The solvent removed in SR-1 is passed together with the additional solvent required for mixing with the light flow from D-1 for further reextraction and settling in D-2. Optionally the system comprising M-2, E-4 and D-2 may be replaced by countercurrent extraction.

### Operating conditions for the process according to the flow diagram in Figure 3

Flow 6 leaves column C-1 at a temperature which generally varies within the range 50 - 115°C. This flow has a solvent content which likewise varies within the range 70 - 95%, most frequently being 80 - 85%. The oil contained in this flow has a polyaromatic hydrocarbons content which varies within the range 4 - 30%.

A counter-solvent such as a light paraffin, e.g. n-heptane (7), is added to this flow and the mixture is cooled to a temperature within the range 10 - 90°C, preferably 20 - 50°C, in exchanger E-2. Optionally flow (7) may be added after the cooling stage in E-2. The cold flow from E-2 passes to mixer M-1 in order to achieve satisfactory contact between the phases and is passed to settler D-1 where a light phase consisting of solvent, counter-solvent and a mixture of hydrocarbons having a PAC content in the range 0.5 - 15%, depending fundamentally on the nature of vacuum distillate 2, separates out. The light flow leaving D-1 is mixed (M-2) with solvent previously cooled in E-3 to a temperature below the boiling point of the most volatile component, preferably 30 - 50°C. Optionally it can be cooled again in exchanger E-4 to the desired settling temperature, generally within the range 15 - 90°C and preferably within the range 15 - 50°C. Flow (17), which is cold, is passed to settler D-2 where a light phase (18) consisting of counter-solvent, solvent and a mixture of hydrocarbons having a low polyaromatic compounds content again settles out and is passed to system SR-2 to remove solvent and counter-solvent.

### Examples of practical embodiments of the invention

The process according to the invention will now be described with reference to the following examples which are offered purely by way of illustration. Examples 4 and 5 are included in the present description for information purposes only.

### Example 1

This example includes the results obtained in the treatment of the mixed extract flow (6) obtained from furfural extraction to obtain SN-600. The outlet temperature of this flow was 85 - 95°C. The flow was cooled at different temperatures in E2 and settled in D-1. The light flow from D-1 was mixed with additional furfural at a higher temperature in M-2. The resulting flow (16) was cooled to the same temperature as in E-2 and settled in D-2. The results obtained were:

These results indicate the advantage of cooling to the minimum temperature possible in E-2 and E-3. A product having a similar PAC content is obtained at 40 and 50°C, but the yield at 40°C is seven points higher than that obtained by cooling and reextracting at 50°C. Likewise, the product obtained at 40°C is more aromatic that that obtained at 50°C.

### Example 2

This example includes the results obtained from the treatment of the mixed extract flow 6 obtained from the furfural extraction of deasphalted vacuum bottoms. The outlet temperature of this flow was 100 - 110°C. The flow was cooled to different temperatures in E2 and settled in D-1. The light flow from D-1 had a PAC content of less than 3% once the solvent had been removed, and it was not reextracted for this reason.

| Experiment no. | 3 | 4 |
|---|---|---|
| Furfural content of the mixed extract flow, % w/w | 92.1 | 92.2 |
| Refractive index of the hydrocarbon phase at 60°C | 1.5483 | 1.5484 |
| PAC content of the hydrocarbon phase, % w/w, IP-346 | 5.4 | 5.5 |
| Separation temperature in D-1, °C | 40 | 50 |
| Yield of raffinate(*)in D-1, % w/w | 54.7 | 47.1 |

| Analysis of the raffinate in D-1 | | |
|---|---|---|
| Furfural content, % w/w | 11.9 | 12.8 |
| Refractive index at 60°C | 1.5260 | 1.5235 |
| Density at 70/4°C | 0.9339 | 0.9306 |
| Aniline point, °C | 74.8 | 78.0 |
| Viscosity at 100°C, cSt | 59.21 | 58.35 |
| Viscosity at 40°C, cSt | 2450 | 2208 |
| Viscosity index | 48 | 55 |
| Pour point, °C, ASTM D-97 | +15 | +18 |
| PAC content, % w/w, IP-346 | 1.1 | 0.9 |
| Sulphur, % w/w, ASTM D-4294 | 3.62 | 3.49 |

| Hydrocarbon composition, ASTM D-2007 | | |
|---|---|---|
| Saturated hydrocarbons, % w/w | 14.8 | 15.9 |
| Polar compounds, % w/w | 9.6 | 10.2 |
| Aromatic hydrocarbons, % w/w | 75.6 | 73.9 |

| | | |
|---|---|---|
| (*): Solvent free base oil | | |

These results show the advantage of cooling to the minimum possible temperature in E-2. A product having a similar PAC content is obtained at 40 and 50°C, but the yield at 40°C is seven points greater than that obtained by cooling and reextracting at 50°C. Likewise the product obtained at 40°C is more aromatic that that obtained at 50°C.

### Example 3

This example includes the results obtained from the treatment of the mixed extract flow, 6, obtained from furfural extraction to obtain a SN-150 base oil. The outlet temperature of this flow was 80°C. The flow was cooled to 40°C in E2 and settled in D-1. The light flow from D-1 was mixed with additional furfural at a higher temperature in M-2. The resulting flow 16 was cooled to the same temperature as in E-2 and settled in D-2. The results obtained were:

| Experiment no. | 5 |
|---|---|
| Furfural content of the mixed extract flow, % w/w | 81.1 |
| Refractive index of the original extract at 70°C | 1.5389 |
| PAC content of the hydrocarbon phase, % w/w, IP-346 | 22 |
| Separation temperature in D-1, °C | 40 |
| Yield of raffinate (*) in D-1, % w/w | 33.0 |

| Analysis of the raffinate in D-1 | |
|---|---|
| Furfural content, % w/w | 10.4 |
| Refractive index at 70°C | 1.4900 |
| Density at 70°C | 0.8806 |
| PAC content, % w/w, IP-346 | 5.8 |

| Reextraction of the light | phase from D-1 |
|---|---|
| Ratio of furfural/light phase from D-1 (w/w) | 2.4/1 |
| Separation temperature in D-2, °C | 40 |
| Yield of raffinate (*) in D-2 % w/w | 78.4 |

| Analysis of the raffinate from D-2 | |
|---|---|
| Furfural content, % w/w | 6.8 |
| Refractive index at 70°C | 1.4782 |
| Density at 70/4°C | 0.8631 |
| Aniline point, °C | 79.4 |
| Viscosity at 100°C, cSt | 5.23 |
| Viscosity at 40°C cSt | 33.38 |
| Viscosity index | 80 |
| PAC content, % w/w | 2.5 |
| Pour point, °C, ASTM D-97 | +15 |
| Sulphur, % w/w, ASTM D-4294 | 1.76 |

| Hydrocarbon composition, ASTM D-2007 | |
|---|---|
| Saturated hydrocarbons, % w/w | 46.9 |
| Polar compounds, % w/w | 1.0 |
| Aromatic hydrocarbons, % w/w | 52.1 |
| OVERALL YIELD | 25.9 |

### Example 4

This example includes the results obtained in treatment of the mixed extract flow, 6, obtained from furfural extraction to obtain SN-600. In this case the results obtained by cooling and reextracting at 40°C are compared with those obtained under similar conditions but with the addition of water to the flow 6. The results obtained were:

| Experiment no. | 6 | 7 |
|---|---|---|
| Furfural content of the mixed extract flow, % w/w | 85.9 | 85.9 |
| Refractive index at 60°C | 1.5640 | 1.5640 |
| PAC content of the hydrocarbon phase, % w/w, IP-346 | 16 | 16 |
| Water added, % w/w (with reference to furfural) | 0 | 1.6 |
| Separation temperature in D-1, °C | 40 | 40 |
| Yield of raffinate ( ∗ ) in D-1, % w/w | 35.0 | 44.3 |

| Analysis of the raffinate from D-1 | | |
|---|---|---|
| Furfural content, % w/w | 10.8 | 11.7 |
| Refractive index at 60°C | 1.5179 | 1.5243 |
| PAC content, % w/w | 3.5 | 4.7 |

| Reextraction of the light phase from D-1 | | |
|---|---|---|
| Ratio of furfural/light phase D-1, w/w | 0.9/1 | 1.7/1 |
| Separation temperature in D-2 | 40 | 40 |
| Raffinate yield ( ∗ ) in D-2, % w/w | 92.5 | 86.0 |

| Analysis of the raffinate from D-2 | | |
|---|---|---|
| Furfural content, % w/w | 10.7 | 11.0 |
| Refractive index at 60°C | 1.5135 | 1.5170 |
| Viscosity at 100°C, cSt | 19.35 | 20.60 |
| Viscosity at 70°C, cSt | 63.30 | 69.92 |
| Viscosity index | 34 | 26 |
| Density at 70/4°C | 0.9138 | 0.9185 |
| Aniline point, °C | 72.8 | 70.0 |
| PCAs, % w/w | 2.7 | 2.8 |
| Overall yield | 32.4 | 38.1 |

| | | |
|---|---|---|
| (*) From solvent-free base. | | |

These results show that the addition of water to the mixed extract from column C-1 (1.6% with respect to solvent) produces an increase of 5 to 6 points in yield of raffinate from D-2 with a PAC content of less than 3%.

### Example 5

This example includes the results obtained from the treatment of the mixed extract flow, 6, obtained from furfural extraction to obtain SN-600. In this case the results obtained by cooling and reextracting at 40°C are compared with those obtained under similar temperature conditions but with the addition of a counter-solvent prior to cooling in E-2. The results obtained were:

| Experiment no. | 1 | 8 |
|---|---|---|
| Furfural content of the mixed extract flow, % w/w | 85.1 | 85.1 |
| Refractive index of the hydrocarbon phase at 60°C | 1.5574 | 1.5574 |
| PAC content of the hydrocarbon phase, % w/w, IP-346 | 16 | 16 |
| Added heptane (ratio of heptane/mixed extract, w/w) | --- | 0.15/1 |
| Separation temperature in D-1, °C | 40 | 40 |
| Yield of raffinate(*) in D-1, % w/w | 43.7 | 61.0 |

| Analysis of the raffinate from D-1 | | |
|---|---|---|
| Furfural + n-heptane content, % w/w | 12.0 | 52.5 |
| Refractive index at 60°C | 1.5143 | 1.5260 |
| PAC content, % w/w, IP-346 | 4.1 | 4.8 |

| Reextraction of the light phase from D-1 | | |
|---|---|---|
| Ratio of furfural/light phase D-1, w/w | 0.73/1 | 1.15/1 |
| Separation temperature in D-2, °C | 40 | 40 |
| Raffinate yield (*) in D-2, % w/w | 93.2 | 88.3 |

| Analysis of the raffinate from D-2 | | |
|---|---|---|
| Furfural + n-heptane content, % w/w | 10.7 | 48.5 |
| Refractive index at 60°C | 1.5124 | 1.5182 |
| Viscosity at 100°C, cSt | 18.75 | 20.29 |
| Viscosity at 70°C, cSt | --- | 67.40 |
| Viscosity index | 48 | 33 |
| Density at 70/4°C | 0.9154 | 0.9210 |
| Aniline point, °C | 72.6 | 66.8 |
| PCAs, % w/w | 2.4 | 2.9 |
| Overall yield | 40.7 | 53.9 |

| | | |
|---|---|---|
| (*) From solvent-free base. | | |

These results show that an increase in yield of approximately 13 points of product having a PAC content of less than 3% is obtained by adding a counter-solvent such as n-heptane to the mixed extract leaving C-1.

### Example 6

This example includes the results obtained from the treatment of the mixed extract flow, 6, obtained from furfural extraction to obtain SN-600. In this case the results obtained by cooling and reextracting at 40°C are compared with those obtained under similar temperature conditions but with removing part of the furfural from the flow 6 in SR-1 before cooling in E-2 and reextracting the light phase from D-1 with additional furfural in order to make up the total furfural/extract ratio used in example 1.

| Experiment no. | 1 | 9 |
|---|---|---|
| Furfural content of the mixed extract flow, % w/w | 85.0 | 85.0 |
| Furfural content of the flow entering E-2 | 85.0 | 75.1 |
| Refractive index of the hydrocarbon phase at 60°C | 1.5574 | 1.5574 |
| PAC content of the hydrocarbon phase, % w/w, IP-346 | 16 | 16 |
| Separation temperature in D-1, °C | 40 | 40 |
| Yield of raffinate (*) in D-1, % w/w | 43.7 | 58.3 |

| Analysis of the raffinate from D-1 | | |
|---|---|---|
| Furfural content, % w/w | 12.01 | 13.2 |
| Refractive index at 60°C | 1.5165 | 1.5281 |
| PAC content, % w/w, IP-346 | 4.1 | 5.8 |

| Reextraction of the light phase from D-1 | | |
|---|---|---|
| Separation temperature in D-2, °C | 40 | 40 |
| Furfural/mixed raffinate, w/w | 0.73/1 | 5.8/1 |
| Raffinate yield (*) in D-2, % w/w | 93.2 | 67.7 |

| Analysis of the raffinate from D-2 | | |
|---|---|---|
| Furfural content, % w/w | 10.7 | 10.7 |
| Refractive index at 60°C | 1.5124 | 1.5099 |
| Density at 70/4°C | 0.9154 | 0.9094 |
| Aniline point, °C | 72.6 | 74.8 |
| Viscosity at 100°C, cSt | 18.75 | 18.05 |
| Viscosity at 70°C, cSt | 58.85 | 56.41 |
| Viscosity at 40°C. cSt | 328.0 | 313.18 |
| Viscosity index | 48 | 46 |
| PAC content, % w/w, IP-346 | 2.4 | 1.8 |

| HYDROCARBON COMPOSITION, ASTM D-2007 | | |
|---|---|---|
| Saturated hydrocarbons, % w/w | 23.5 | --- |
| Polar compounds, % w/w | 5.3 | --- |
| Aromatic hydrocarbons, % w/w | 71.2 | --- |
| Overall yield of low PAC content raffinate, % w/w | 40.7 | 39.5 |

| | | |
|---|---|---|
| (*) Solvent-free base. | | |

These results show that distribution of the solvent into equal parts in D-1 and D-2 makes it possible to obtain a raffinate with a reduced PAC content without the need to use additional solvent.

### Example 7

This example contains the results obtained in the treatment of the flow of mixed extract 6, resulting from the extraction with furfural to obtain SN-600. In this case, the results obtained by cooling and re-extracting at 40°C are compared with ones obtained in similar conditions of temperature but adding a hydrocarbonated stream with IBP greater than 200°C to the flow of mixed extract 6, before cooling at E-2 and extracting the light phase from D-1 with additional furfural to reduce the PCA content to below 3%.

| Experiment no. | 1 | 10 |
|---|---|---|
| Furfural content of the mixed extract flow, % w/w | 85.0 | 85.0 |
| Added hydrocarbonated stream (w/w mixed extract) | 0 | 0.105/1 |
| I. Refraction at 60°C of the hydrocarbon phase | 1.5574 | 1.5271 |
| PAC content of the hydrocarbon phase, % w/w, IP-346 | 16 | 11.1 |
| Separation temperature in D-1, °C | 40 | 40 |
| Yield of raffinate(*)in D-1, % w/w | 43.7 | 70.8 |

| Analysis of the raffinate from D-1 | | |
|---|---|---|
| Furfural content, % w/w | 12.01 | 8.0 |
| I. Refractive index at 60°C | 1.5165 | 1.4987 |
| PAC content, % w/w, IP-346 | 4.1 | 3.1 |

| Reextraction of the light phase from D-1 | | |
|---|---|---|
| Separation temperature in D-2, °C | 40 | 40 |
| Furfural/mixed raffinate, w/w | 0.73/1 | 0.5/1 |
| Raffinate yield (*) in D-2, % w/w | 93.2 | 96.8 |

| Analysis of the raffinate from D-2 | | |
|---|---|---|
| Furfural content, % w/w | 10.7 | 7.1 |
| I. Refractive index at 60°C | 1.5124 | 1.4972 |
| Density at 70/4°C | 0.9154 | 0.8885 |
| Aniline point, °C | 72.6 | 91.4 |
| Viscosity at 100°C, cSt | 18.75 | 15.11 |
| Viscosity at 40°C, cSt | 328.0 | 200.2 |
| | | |
| Viscosity index | 48 | 67 |
| PAC content, % w/w, IP-346 | 2.4 | 2.5 |

| HYDROCARBON COMPOSITION, ASTM D-2007 | | |
|---|---|---|
| Saturated hydrocarbons, % w/w | 23.5 | 46.1 |
| Polar compounds, % w/w | 5.3 | 4.0 |
| Aromatic hydrocarbons, % w/w | 71.2 | 49.9 |
| Overall yield of low PAC content raffinate, % w/w | 40.7 | 68.6 |

| | | |
|---|---|---|
| (*) Solvent-free base. | | |

These results prove that the addition of a hydrocarbonated stream (IBP greater than 200°C) allows increasing the production of aromatic oil with low PCA content without notable inrease of furfural required in the re-extraction of the raffinate obtained in the first settling step.

Analyses of an oil B obtained from a mixed SN-600 extract according to this invention are shown in the table below. In this table the results of the analyses are compared with those for an extract from the state of the art (A).

The results of the analyses of an oil D obtained from a mixed deasphalted vacuum bottoms extract according to this invention are shown. The results are compared with those corresponding to an extract from the state of the art (C).

| | SN-600 extract | | Deasphalted oil extract | |
|---|---|---|---|---|
| OIL | A | B | C | D |
| PAC content, % w/w, IP-346 | 16 | 2.6 | 5.5 | 1.5 |
| Mutagenicity index (MI) (modified Ames test) | >1 | 0.2 | --- | 0 |
| Viscosity at 100°C, cSt, ASTM D-445 | 33.6 | 19.54 | 71.02 | 51.22 |
| Flash point, open cup, °C, ASTM D-92 | 276 | 278 | 302 | 318 |
| Loss on evaporation, 3 0.04 hours, 163°C, % w/w | | 0.01 | 0.04 | 0.01 |

| Hydrocarbon composition, ASTM D-2007 | | | | |
|---|---|---|---|---|
| Saturated hydrocarbons, % w/w | 10.7 | 26.5 | 13.9 | 23.2 |
| Polar compounds, % w/w | 11.0 | 5.7 | 12.1 | 10.5 |
| Aromatic hydrocarbons, % w/w | 78.3 | 67.8 | 74 | 66.3 |

| DISTILLATION, modified ASTM D-2887 | | | | |
|---|---|---|---|---|
| IBP | 378 | 382 | 464 | 483 |
| 5% | 435 | 442 | 507 | 515 |
| 50% | 500 | 506 | 584 | 584 |
| 90% | 547 | 548 | 661 | 662 |
| 95% | 562 | 561 | 682 | 685 |
| FBP | 599 | 596 | 725 | 726 |

In the table below PAH contents according to the US EPA 8270/95 method in products obtained using the process according to this invention are compared with those corresponding to present-day aromatic extracts.

### Industrial application of the invention

One of the objectives of this invention is to develop aromatic oils having a low PAC content which will not be regarded as potentially carcinogenic for application as rubber extenders.

Three samples of rubber using a typical formulation for tyres have been prepared with a view to comparing the properties of rubbers formulated using these oils with a low PAC content and rubbers formulated with aromatic oils having a high PAC content.

| FORMULATION | |
|---|---|
| Component | Parts by weight |
| SBR 1502 (Krylene 1502) | 60 |
| High cis polybutadiene (PB 1202) | 40 |
| N-234 carbon black (ISAF-HS) | 70 |
| Aromatic oil | 40 |
| Zinc oxide | 3 |
| Stearic acid | 2 |
| Santoflex 13 (N-(1,3-dimethylbutyl-N'-phenyl-p-phenylenediamine) | 1 |
| HS antioxidant (Poly(2,2,4-trimethyl-1,2-dihydroquinoline)) | 2 |
| Redezon (Repsol antiozone wax) | 3 |
| Rubenamide C™ (N-cyclohexylbenzothiacyl-sulphenamide) | 1 |
| Sulphur | 1.75 |

Three samples were prepared, each with one type of oil (A, B, D) in a cylinder mixer 30 cm long having a friction ratio of 1:1.14. The same order of addition and the same mixing time were used in the preparation of the samples. The vulcanization temperature was 150°C in all three cases.

The table below includes the properties of the vulcanizates:

| Mixtures | Mixture A | Mixture B | Mixture D |
|---|---|---|---|
| Oil used | A | B | D |
| Property | | | |
| Shore hardness A | 51.0 | 51.9 | 52.7 |
| Resilience, % | 30 | 30 | 28.5 |
| 100% deformation force, MPa | 1.13 | 1.17 | 1.10 |
| 300% deformation force, MPa | 4.50 | 4.67 | 4.23 |
| 500% deformation force, MPa | 10.51 | 10.75 | 9.41 |
| Tensile strength, MPa | 16.31 | 16.32 | 17.14 |
| Elongation on fracture, % | 694 | 680 | 769 |
| Tear resistance, N | 55.3 | 53.7 | 57.2 |

These results show that when state-of-the-art oil (A) is replaced by oils obtained in accordance with this invention (B, D) rubbers with very similar properties are obtained. Nevertheless, it is not the purpose of this patent to provide a formulation, but only to compare the rubbers formulated under identical conditions using state-of-the-art oils and those obtained in accordance with this invention.

## Claims

1. Process for obtaining aromatic oils with a polycyclic aromatic compounds content of less than 3% (IP-346) from the mixed extract flow obtained in the manufacture of lubricant base oils, a flow which contains a polar solvent in a rate between 70 and 95 %, preferably of the group comprising phenol, furfural and N-methyl-2-pyrrolidone, preferably furfural, **characterized in that** it comprises the stages of:
a) cooling the flow of mixed extract to render non-polyaromatic components insoluble,
b) settling to bring about separation of the phases,
c) conducting the heavy phase obtained from the settling in step b) to a solvent recovery system,
d) total or partial redissolution in solvent of the light phase obtained from the settling in stage b),
e) cooling to effect separation of the non-polyaromatic components,
f) settling to bring about separation of the phases,
g) conducting the heavy phase obtained from the settling in step f) to the solvent recovery system of step c)
h) recovering the light phase having a low polyaromatic compounds content obtained from the settling in step f),
i) passing said light phase to a system for the recovery of the solvent, and
j) recycling the solvent recovered in steps c), g) and i) to the process.

2. Process for obtaining aromatic oils with a polycyclic aromatic compounds content of less than 3% (IP-346) from the mixed extract flow, originating from the solvent extraction of a deasphalted vacuum bottom, obtained in the manufacture of lubricant base oils, a flow which contains a polar solvent in a rate between 70 and 95 %, preferably of the group comprising phenol, furfural and N-methyl-2-pyrrolidone, preferably furfural, **characterized in that** it comprises the stages of:
a) cooling the flow of mixed extract to render non-polyaromatic components insoluble,
b) settling to bring about separation of the phases,
c) conducting the heavy phase obtained from the settling in step b) to a solvent recovery system,
d) passing directly the light phase obtained in step b) to a system for the recovery of the solvent, and
e) recycling the solvent recovered in steps c) and d) to the process.

3. Process according to any of claims 1 or 2, **characterized in that** an antisolvent such as water is added to the starting mixed extract flow to increase selectivity for polyaromatic compounds.

4. Process according to claim 3, **characterized in that** the quantity of anti-solvent added varies between 0.5 and 10%, and preferably between 0.5 and 5% and especially between 1 and 2.5%.

5. Process according to Claims 1 and 4, **characterized in that** the quantity of additional solvent in relation to the flow of the hydrocarbon phase in the mixed extract flow is always less than 1.5:1 and preferably less than 1:1.

6. Process according to Claims 1 or 2, **characterized in that** some of the solvent contained in the mixed extract flow is removed before the cooling stage in order to achieve an approximately 50%. distribution of solvent in the stages prior to settling.

7. Process according to Claims 1 or 2, **characterized in that** a hydrocarbon stream, having an initial boiling point at 101 kPa (760 mm) Hg greater than 200°C, preferably greater than 300°C, is added to the starting mixed extract flow to regulate the solvent/solute rate and increase the production capacity.

8. Process according to claim 7, **characterized in that** the added hydrocarbon stream is a product obtained in any of the vaccuum destilation processes of the atmospheric residue, extraction with solvent, dewaxing or deasphalting.

9. Process according to Claims 1 or 2, **characterized in that** a counter-solvent is added before the first cooling stage to increase the selectivity of the solvent contained in the mixed extract flow.

10. Process according to Claim 9, **characterized in that** the counter-solvent is a hydrocarbon flow with a maximum boiling point of less than 160°C, preferably less than 140°C.

11. Process according to any one of Claims 1, 2, 3, 6, 7 and 9, **characterized in that** the cooling temperature before the settling stages lies within the range 10 - 90°C, preferably within the range 10 - 60°C and in particular within the range 20 - 50°C.

## Patentansprüche

1. Verfahren zur Herstellung aromatischer Öle mit einem Gehalt an polycyclischen Aromaten von weniger als 3% nach IP-346 aus dem bei der Herstellung von Grundölen für Schmieröle anfallenden Mischextraktstrom, der ein polares Lösungsmittel in einem Anteil zwischen 70 und 95%, vorzugsweise aus der Gruppe Phenol, Furfural und N-Methyl-2-pyrrolidon und vorzugsweise Furfural, enthält, **dadurch gekennzeichnet, daß** man:
a) den Mischextraktstrom abkühlt, damit die nicht polyaromatischen Komponenten unlöslich werden,
b) zwecks Phasentrennung absetzen läßt,
c) die aus dem Absetzen in Schritt b) erhaltene schwere Phase einem Lösungsmittelrückgewinnungssystem zuführt,
d) die aus dem Absetzen in Schritt b) erhaltene leichte Phase ganz oder teilweise wieder in Lösungsmittel löst,
e) zur Abtrennung der nicht polyaromatischen Komponenten abkühlt,
f) zwecks Phasentrennung absetzen läßt,
g) die aus dem Absetzen in Schritt f) erhaltene schwere Phase dem Lösungsmittelrückgewinnungssystem von Schritt c) zuführt,
h) die aus dem Absetzen in Schritt f) erhaltene leichte Phase mit niedrigem Gehalt an polyaromatischen Verbindungen zurückgewinnt,
i) die leichte Phase einem Lösungsmittelrückgewinnungssystem zuführt und
j) das in den Schritten c), g) und i) zurückgewonnene Lösungsmittel in das Verfahren zurückführt.

2. Verfahren zur Herstellung aromatischer Öle mit einem Gehalt an polycyclischen Aromaten von weniger als 3% nach IP-346 aus dem aus der Lösungsmittelextraktion eines entasphaltierten Vakuumrückstands stammenden, bei der Herstellung von Grundölen für Schmieröle anfallenden Mischextraktstrom, der ein polares Lösungsmittel in einem Anteil zwischen 70 und 95%, vorzugsweise aus der Gruppe Phenol, Furfural und N-Methyl-2-pyrrolidon und vorzugsweise Furfural, enthält, **dadurch gekennzeichnet, daß** man:
a) den Mischextraktstrom abkühlt, damit die nicht polyaromatischen Komponenten unlöslich werden,
b) zwecks Phasentrennung absetzen läßt,
c) die aus dem Absetzen in Schritt b) erhaltene schwere Phase einem Lösungsmittelrückgewinnungssystem zuführt,
d) die in Schritt b) erhaltene leichte Phase direkt einem Lösungsmittelrückgewinnungssystem zuführt und
e) das in den Schritten c) und d) zurückgewonnene Lösungsmittel in das Verfahren zurückführt.

3. Verfahren nach Anspruch 1 oder 2, **dadurch gekennzeichnet, daß** man zur Erhöhung der Selektivität für polyaromatische Verbindungen dem als Edukt dienenden Mischextraktstrom ein Antilösungsmittel wie Wasser zusetzt.

4. Verfahren nach Anspruch 3, **dadurch gekennzeichnet, daß** man das Antilösungsmittel in einer Menge zwischen 0,5 und 10%, vorzugsweise zwischen 0,5 und 5% und insbesondere zwischen 1 und 2,5% zusetzt.

5. Verfahren nach den Ansprüchen 1 und 4, **dadurch gekennzeichnet, daß** die Menge an zusätzlichem Lösungsmittel, bezogen auf den Strom der Kohlenwasserstoffphase in dem Mischextraktstrom, immer unter 1,5:1 und vorzugsweise unter 1:1 liegt.

6. Verfahren nach Anspruch 1 oder 2, **dadurch gekennzeichnet, daß** man vor dem Abkühlschritt einen Teil des in dem Mischextraktstrom enthaltenen Lösungsmittels entfernt, damit sich in den Stufen vor dem Absetzen eine ungefähr 50%ige Verteilung von Lösungsmittel ergibt.

7. Verfahren nach Anspruch 1 oder 2, **dadurch gekennzeichnet, daß** man dem als Edukt dienenden Mischextraktstrom zur Regulierung des Verhältnisses von Lösungsmittel zu Gelöstem und zur Erhöhung der Produktionskapazität einen Kohlenwasserstoffstrom mit einem Siedebeginn bei 101 kPa (760 mm Hg) von mehr als 200°C und vorzugsweise mehr als 300°C zusetzt.

8. Verfahren nach Anspruch 7, **dadurch gekennzeichnet, daß** es sich bei dem zugesetzten Kohlenwasserstoffstrom um ein bei einem Verfahren der Vakuumdestillation des atmosphärischen Rückstands, bei der Lösungsmittelextraktion, Entparaffinierung oder Entasphaltierung erhaltenes Produkt handelt.

9. Verfahren nach Anspruch 1 oder 2, **dadurch gekennzeichnet, daß** man vor dem ersten Abkühlschritt zur Erhöhung der Selektivität des in dem Mischextraktstrom enthaltenen Lösungsmittels ein Gegenlösungsmittel zusetzt.

10. Verfahren nach Anspruch 9, **dadurch gekennzeichnet, daß** es sich bei dem Gegenlösungsmittel um einen Kohlenwasserstoffstrom mit einem maximalen Siedepunkt von weniger als 160°C und vorzugsweise weniger als 140°C handelt.

11. Verfahren nach einem der Ansprüche 1, 2, 3, 6, 7 und 9, **dadurch gekennzeichnet, daß** die Abkühlungstemperatur vor den Absetzschritten im Bereich von 10-90°C, vorzugsweise im Bereich von 10-60°C und insbesondere im Bereich von 20-50°C liegt.

## Revendications

1. Procédé pour l'obtention d'huiles aromatiques ayant une teneur en composés aromatiques polycycliques de moins de 3 % (IP-346) à partir du courant d'extrait mélangé obtenu dans la fabrication d'huiles de base de type lubrifiant, un courant qui comprend un solvant polaire selon un taux de 70 à 95 %, de préférence du groupe comprenant le phénol, le furfural et la N-méthyl-2-pyrrolidone, de préférence le furfural, **caractérisé en ce qu'**il comprend les étapes consistant à :
a) refroidir le courant d'extrait mélangé pour rendre les composant non polyaromatiques insolubles,
b) décanter pour entraîner la séparation des phases,
c) transporter la phase lourde obtenue lors de la décantation de l'étape b) vers un système de récupération de solvant,
d) re-dissoudre totalement ou partiellement dans un solvant la phase légère obtenue lors de la décantation de l'étape b),
e) refroidir pour effectuer la séparation des composants non polyaromatiques,
f) décanter pour entraîner la séparation des phases,
g) transporter la phase lourde obtenue lors de la décantation de l'étape f) vers le système de récupération de solvant de l'étape c),
h) récupérer la phase légère, ayant une faible teneur en composés aromatiques polycycliques, obtenue lors de la décantation de l'étape f),
i) passer ladite phase supérieure vers un système pour la récupération du solvant, et
j) recycler le solvant récupéré dans les étapes c), g) et i) vers le traitement.

2. Procédé pour l'obtention d'huiles aromatiques ayant une teneur en composés aromatiques polycycliques de moins de 3 % (IP-346) à partir du courant d'extrait mélangé, provenant de l'extraction de solvant d'un fond sous vide déasphalté, obtenu dans la fabrication d'huiles de base de type lubrifiant, un courant qui comprend un solvant polaire dans une plage allant de 70 à 95 %, de préférence du groupe le phénol, le furfural et la N-méthyl-2-pyrrolidone, de préférence le furfural, **caractérisé en ce qu'**il comprend les étapes consistant à :
a) refroidir le courant d'extrait mélangé pour rendre les composant non polyaromatiques insolubles,
b) décanter pour entraîner la séparation des phases,
c) transporter la phase lourde obtenue lors de la décantation de l'étape b) vers un système de récupération de solvant,
d) passer directement la phase légère vers un système pour la récupération du solvant, et
e) recycler le solvant récupéré dans les étapes c) et d) vers le traitement.

3. Procédé selon la revendication 1 ou 2, **caractérisé en ce qu'**un anti-solvant, tel que l'eau, est ajouté au courant d'extrait mélangé de départ pour augmenter la sélectivité pour les composés polyaromatiques.

4. Procédé selon la revendication 3, **caractérisé en ce que** la quantité d'anti-solvant ajouté varie dans la plage allant de 0,5 à 10 %, de préférence allant de 0,5 à 5 % et spécifiquement allant de 1 à 2,5 %.

5. Procédé selon la revendication 1 ou 4, **caractérisé en ce que** la quantité de solvant supplémentaire par rapport au courant de la phase d'hydrocarbure dans le courant d'extrait mélangé est toujours inférieure à 1,5:1, et de préférence inférieure à 1:1.

6. Procédé selon la revendication 1 ou 2, **caractérisé en ce qu'**une partie du solvant compris dans le courant d'extrait mélangé est retirée avant l'étape de refroidissement afin d'obtenir une distribution d'environ 50 % de solvant dans les étapes avant la décantation.

7. Procédé selon la revendication 1 ou 2, **caractérisé en ce qu'**un courant d'hydrocarbure, ayant un point d'ébullition initial à 101 kPA (760 mm de Hg) supérieur à 200°C, de préférence supérieur à 300 C, est ajouté au courant d'extrait mélangé de départ pour réguler la taux solvant/soluté et augmenté la capacité de production.

8. Procédé selon la revendication 7, **caractérisé en ce que** le courant d'hydrocarbure ajouté est un produit obtenu dans n'importe quel procédé de distillation sous vide de résidus atmosphériques, extraction avec un solvant, débarrassage des cires ou déasphaltage.

9. Procédé selon la revendication 1 ou 2, **caractérisé en ce que** le solvant opposé est ajouté avant la première étape de refroidissement pour augmenter la sélectivité du solvant compris dans le courant d'extrait mélangé.

10. Procédé selon la revendication 9, **caractérisé en ce que** le solvant opposé est un courant d'hydrocarbure ayant un point d'ébullition maximal de moins de 160 °C, de préférence de moins de 140 °C.

11. Procédé selon l'une quelconque des revendications 1, 2, 3, 6, 7 et 9, **caractérisé en ce que** la température de refroidissement avant les étapes de décantation est comprise dans la plage allant de 10 à 90 °C, de préférence allant de 10 à 60 °C et en particulier allant de 20 à 50°C.
